

## UNITED STATES PATENT OFFICE

2,646,374

## TEXTILE INTERLINER FABRIC FOR GARMENTS AND METHOD OF MAKING THE SAME

Robert H. Gillespie, Walpole, Mass., assignor to  
The Kendall Company, Boston, Mass., a corporation of Massachusetts

No Drawing. Application February 14, 1950,  
Serial No. 144,203

7 Claims. (Cl. 117—161)

1

The present invention relates to coated fabrics and more particularly to an interliner fabric adapted to be bonded by heat and pressure to a facing fabric to form semi-stiff articles of apparel such as collars, cuffs and shirt bosoms, and to the method of making the same.

Articles of apparel of this type have been known; for example, there have been on the market for many years men's shirts with attached collars containing a resin-coated interliner fabric to provide a collar which is easy to iron and which does not require starching when laundered and yet remains free from wrinkles when worn.

Notwithstanding the obviously great advantages of a collar of this character, such collars as the prior art has heretofore been able to provide have not been wholly satisfactory. One of the worst defects of such collars is their initial stiffness and boardiness. Another serious defect is the substantial change in flexibility which occurs upon repeated laundering, so that the customer who has selected a shirt in the store on the basis of the hand and feel of the collar soon finds that the collar has become too stiff or too soft and is discouraged from again buying a fused-collar shirt.

I have found that such a collar, and similarly cuffs, shirt bosoms and other semi-stiff articles of apparel, to be widely acceptable must satisfy a large number of exacting and apparently irreconcilable requirements. A collar, for example, must not be objectionably stiff and boardy, and yet must be sufficiently firm not to wrinkle when worn. Also, the degree of flexibility or stiffness must remain substantially uniform throughout the useful life of the garment, notwithstanding repeated laundering and repeated ironing at temperatures of 250° to 350° F. This provision of a desirable degree of initial flexibility and softness, and maintenance of this optimum value throughout the life of the garment has until now presented an unsolvable problem.

The interliner material, further, must be one which is capable of being fused to facing fabrics at the temperatures and pressures available to the shirt manufacturer to form a permanent bond strong enough to resist ply-separation in repeated cycles of wear and laundering and yet should not permit the adhesive to strike through or to bleed objectionably through the facing ma-

2

terial, at these temperatures or at ironing temperatures. Otherwise, the stiffness will change with each ironing and/or the collar will be discolored or disfigured. In addition, the collar, both interliner and facing united thereto, should be porous and permeable to perspiration and to the liquids employed in laundering.

It is an object of my invention to provide an apparel interliner material of the character indicated which will satisfy all of the foregoing requirements. Another object of the invention is to provide an interliner material which will provide wrinkle-resistant collars and the like having an initial desirable softness and flexibility and retaining this desirable quality substantially unchanged throughout their useful life. A further object of the invention is to provide such interliner material yielding garments which are comfortable to wear and are porous and permeable to perspiration and to washing liquids. It is a further object of this invention to provide an interliner material, which, when fused to a facing fabric, will provide a laminate that is substantially resistant to ply separation on repeated laundering. It is a further object of this invention to provide an interliner material that may be fused to a facing fabric on conventional equipment but which after laundering does not bleed or strike through at temperatures encountered in laundering presses.

In accordance with the invention, I coat a conventional interliner fabric, typically a 64 x 56 bleached cotton print cloth, with a mixture of separately-polymerized resins comprising a liquid dispersion of a high-molecular-weight vinyl chloride polymer (inclusive of copolymers) having an average molecular weight above about 20,000 and a combined vinyl chloride content in excess of 90% by weight of the polymer, in the continuous phase of a solution of a low-molecular-weight vinyl chloride polymer (inclusive of copolymers) having an average molecular weight between about 5,000 and 16,000 and a combined vinyl chloride content in excess of about 60% by weight of the polymer. The molecular weights referred to herein are determined by Staudinger's method (Ind. Eng. Chem., vol. 28, p. 1152, 1936). In addition to these polymers and the solvent, my coating composition includes in the continuous phase of the solution two types of plasticizers,

one a non-leachable plasticizer which is not removed from the garment to any significant extent by repeated laundering, and the other a leachable plasticizer which is removed in laundering in an appreciable amount.

After the coating is applied to the fabric the solvent is removed by evaporation, leaving a smooth, continuous film containing the high and low molecular weight resin components and plasticizer in two distinct solid phases.

The combination of polymers and the combination of plasticizers, which I employ, together with dispersion of the high-molecular-weight polymer in the low-molecular-weight polymer, provide a composition which does not bleed during the operation of compositing the interliner with the facing fabric or in subsequent laundering and ironing, but which nevertheless can be fused by the shirt manufacturer, at the temperatures and pressures available with conventional equipment, to give an adhesive bond between the interliner and facing fabric which is adequately strong, in excess of 3 pounds per square inch, and is permanent in the sense that it endures, without ply separation, beyond the useful life of the garment.

During the fusing operation performed by the shirt manufacturer, the low molecular weight resin component of my coating composition which contains the preponderance of plasticizer, softens readily, effecting an adhesive bond between the interliner and the facing fabric and concurrently having a fluxing action on the high molecular weight resin component. Before fusing, the softening point of the composition is close to that of the plasticized low molecular weight resin component. After fusing, the softening point of the composition is significantly increased, due, it is believed, to migration of plasticizer and low molecular weight resin into high molecular weight resin particles, forming a more homogeneous mixture. Consequently the interliner is less likely to bleed during commercial ironing operations during laundering, which frequently involve higher temperatures than the fusing process. This increase in softening temperature has been demonstrated experimentally by comparative tests of interliner fabric-facing fabric bond strengths with and without pre-heating of the interliner fabric before fusing. The pre-heated interliner showed a 40% reduction in bond strength, indicating that the pre-treatment had significantly raised the softening temperature of the mass.

The resultant interliner, when incorporated in a collar or the like, produces a soft and flexible but wrinkle-resistant garment which softness and wrinkle resistance remain substantially the same throughout the lifetime of the garment. Collars formed from the resultant interliner have tip stiffness values (as hereinafter defined) of between 5 and 20 grams, as contrasted with values of the order of 30 grams characteristic of the prior art. In addition, and due chiefly, it is believed, to the removal of the leachable plasticizer during laundering, the resultant collar has a marked permeability and moisture transferability. This permeability coupled with the retention of substantially the initial softness and flexibility is a marked contribution in the art and is achieved by the inclusion of the two types of plasticizers.

The leachable plasticizer, in addition to its other functions, contributes to the initial flexibility and softness of the material. Any de-

crease in flexibility and softness resulting from loss of this plasticizer during early launderings of the garment is, I believe, offset by the softening effect of laundering. The inclusion of the leachable plasticizer lowers the softening temperature of the mass to facilitate combining of the interliner and facing fabric. On the other hand, I believe, removal of the leachable plasticizer inhibits bleeding during successive laundry pressings by increasing the softening temperature of the mass.

As an illustration of the presently preferred interliner material and process for its manufacture the following example is given.

#### Example

160 lbs. of acetone, 31 lbs. of di(2-ethyl hexyl) phthalate (non-leachable plasticizer) and 8 lbs. of ethyl phthalyl ethyl glycolate (leachable plasticizer) are placed in a 55 gal. tin-lined drum provided with a stirring paddle consisting of a stainless steel shaft and three-bladed propellers at the top, bottom and middle of the shaft. The stirrer is started and 27 lbs. of a low-molecular-weight copolymer of vinyl chloride and vinyl acetate (Vinylite VYHH) wherein the vinyl chloride and vinyl acetate are combined in the proportions of about 87% vinyl chloride to 13% vinyl acetate, having an average molecular weight between about 9,000 and 12,000 are added with continued stirring. At the end of one hour all of the polymer is in solution and the mass is of a smooth consistency. With continued stirring, 50 parts of an emulsion-polymerized vinyl chloride copolymer (Vinylite VYNV), average molecular weight about 24,000 and containing vinyl chloride and vinyl acetate combined in the ratio of about 95:5, are added. The high-molecular-weight polymer is not dissolved but is slightly swollen and is dispersed in the low-molecular-weight copolymer - acetone solution. Care is taken to prevent the temperature of the mass from rising above 95° F. At the end of one hour the mass is a smooth dispersion in which the high-molecular-weight polymer is in the disperse phase. A 64 x 56 bleached starched cotton print cloth is coated with the dispersion, applying on each side 0.85 oz./sq. yd. by means of a single sharp-knife doctor blade, completely filling the interstices, followed by a second coat on each side of 1.25 oz./sq. yd. The total coating weight is 4.20 oz./sq. yd., approximately equally divided between the two sides. Shirt collars were constructed by combining interliners cut from the resulting fabric with outer plies of a facing fabric of 136 x 60 combed yarn broadcloth, using a Model 722 Prosperity fusing press operating at 90 lbs. per square inch steam pressure, and 70 lbs. per square inch air pressure for a twenty second dwell period. These collars showed an initial tip stiffness of 10 grams (as measured by the test hereinafter described) and a bond strength in excess of 4 pounds per inch. Sample collars were subjected to repeated wear and laundering tests and the tip stiffness measured at intervals. During the useful life of the collar no ply separation occurred and the tip stiffness remained between 8 and 12 grams.

As the high-molecular-weight polymer I may employ a vinyl chloride polymer or a copolymer of vinyl chloride with a polymerizable olefinic compound such as vinyl acetate, vinyl propionate, diethyl fumarate, acrylonitrile, vinylidene chloride, maleate esters such as dibutyl maleate and dimethyl maleate, and acrylate esters such as

ethyl acrylate, methyl acrylate, propyl acrylate and methyl methacrylate. Such high-molecular-weight vinyl chloride polymers are characterized by their insolubility and in commercial practice are formed by emulsion polymerization. In producing the products of this invention I have found that the ratio of high-molecular-weight polymer to low-molecular-weight polymer can be from 1:1 to 6:1 by weight. Typical commercial products contain these polymers in the ratio 1.5:1 to 3:1.

The low-molecular-weight polymer may be a copolymer of vinyl chloride with any of the olefinic compounds mentioned above.

Instead of the acetone of the example, I may use any solvent or solvent mixture which will dissolve the low-molecular-weight polymer but will not dissolve, although it may swell, the high-molecular-weight polymer, such as the mixtures of organic liquids customarily employed in the art for forming vinyl chloride organosols, i. e., a mixture of a dispersant, such as acetone, and a diluent such as toluene, xylene or other liquid aromatic hydrocarbon. I prefer to omit the hydrocarbon and use one or more alkyl ketones having the general formula



wherein  $R_1$  and  $R_2$  are alkyl groups selected from the class consisting of methyl, ethyl, n-propyl, isopropyl and isobutyl, principally because of the higher solids content for a given viscosity which I have found that these liquids provide. Of this group, the preferred member is acetone.

In mixing the coating mass I employ sufficient organic liquid to produce a coating medium of a fluidity that will allow easy application to the base fabric by conventional means. Typical compositions contain 30% to 75% by weight of acetone or its equivalent.

Instead of the stirring technique of the example, any appropriate procedure known in the art may be employed for dispersing the high-molecular-weight polymer in the low-molecular-weight copolymer, such as ball-milling, roller-milling, etc.

As the non-leachable plasticizer, I prefer di(2-ethyl hexyl) phthalate because, in addition to its resistance to removal by laundering, it provides, I believe, additional bond strength. I may use, however, any other compatible plasticizer which is resistant to laundering to a degree comparable with di(2-ethyl hexyl) phthalate.

As a measure of leachability of the plasticizer, I have adopted the weight loss resulting from washing of dried films 0.015" thick formed from the polymers of my composition containing 33% of the plasticizer to be evaluated. In this test the films are washed in an agitated aqueous solution containing 0.2% by weight of a good grade of laundry soap and 0.2% by weight of sodium carbonate for a period of one hour at 140° F. For the purpose of my invention, a weight loss of less than 5% of the film indicates that the plasticizer is satisfactory as a non-leachable plasticizer. A weight loss greater than 5% indicates that the plasticizer is satisfactory for use as a leachable plasticizer in my composition.

Typical non-leachable plasticizers, in addition to di(2-ethyl hexyl) phthalate are:

Tricresyl phosphate

Saturated polyester (Paraplex G-50)

Ethyl butyl phthalate

Butyl benzyl phthalate (Santicizer 160)

Butyl phthalyl butyl glycolate (Santicizer B-16)  
Dibutoxy ethyl phthalate (Kronisol)  
Diethyl sebacate

Typical plasticizers which I have found to be satisfactory as the leachable plasticizer of my composition are:

Dimethoxy ethyl phthalate (Methox)  
Diethoxy ethyl phthalate (Ethox)  
Ethyl phthalyl ethyl glycolate (Santicizer E-15)  
Triethyleneglycol di-2-ethyl hexoate (Flexol GO)  
Diethyleneglycol monoethyl ether phthalate

I incorporate a total plasticizer content between about 37% and 58%, by weight of the total polymer content, of which plasticizer as much as 70% can be of the leachable type. Typical products of this invention contain from 5% to 60% leachable plasticizer.

Tip stiffness as used herein is defined as the number of grams required to bend a definite area of the collar through an angle of 30° in the Saxl Stiffness Testing machine, Model No. 201, manufactured by Saxl Instrument Co., Providence, R. I., set at a 3 cm. gap between the fabric-clamp edge and the fabric knife edge. The Saxl apparatus, a machine for testing the flexibility of textiles, consists of a beam balance with a fabric knife edge on one side of the beam. The collar tip rests on the fabric knife edge. The load scale is located on the other side of the balance beam. The collar is held in a clamp which can be rotated to measure the angle through which the collar tip is bent. The collar area which extends past the clamp, i. e., the collar tip, is that enclosed by a triangle, marked by a template, which is 2 1/8" along the clamp edge and 2 3/8" and 2 1/4" along the other two sides. A test is made by determining the angle of bending required to bring the balance to zero when loaded by each of two arbitrarily selected weights. The load is placed on the balance beam while in the arrested position. The beam is lowered onto its knife edge and simultaneously the collar tip is bent as rapidly as possible to bring the balance to zero. The angle of bending required to zero the balance is quickly read and the fabric clamp returned to a zero bending angle as rapidly as possible. This procedure is repeated under the second selected load. In this manner, the collar tip is placed under stress the minimum length of time and resilience and relaxation effects are held to a minimum. The number of grams required to bend the collar tip through an angle of 30° is then found by plotting load versus bending angle for the two points determined, connecting the two points with a straight line and reading the number of grams from the graph at the junction of the drawn line with the 30° angle line.

Pigments, dyes, heat stabilizers, anti-blocking agents, etc., may be incorporated in the composition as desired.

Where the term "bond strength" is used in this application, I intend it to mean the force in pounds required to peel a facing ply from a strip of the laminate one inch wide.

Coating compositions and methods of making them disclosed herein are claimed in my copending application Serial No. 276,439 filed March 13, 1952, as a continuation-in-part of my prior application Serial No. 144,204 filed February 14, 1950, now abandoned.

I claim:

1. An interliner fabric adapted to be bonded

by heat and pressure to a face fabric to form washable wrinkle-resistant articles of apparel such as collars, cuffs, shirt bosoms and the like characterized by a desirable initial softness and flexibility persisting substantially throughout the life of the article of apparel, comprising a fabric coated with a mixture of separately-polymerized synthetic organic resins comprising 1 to 6 parts of a high-molecular-weight emulsion-polymerized vinyl chloride polymer having an average molecular weight above about 20,000 and a combined vinyl chloride content in excess of 90% by weight of the polymer, dispersed as a distinct undissolved solid phase in 1 part of a low-molecular-weight vinyl chloride polymer having an average molecular weight between about 5000 and 16000 and a combined vinyl chloride content in excess of about 60% by weight of the polymer, and a plasticizer in an amount between about 37% and 58% by weight of the total polymer content.

2. An interliner fabric adapted to be bonded by heat and pressure to a face fabric to form washable wrinkle-resistant articles of apparel such as collars, cuffs, shirt bosoms and the like characterized by a desirable initial softness and flexibility persisting substantially throughout the life of the article of apparel, comprising a fabric coated with a mixture of separately-polymerized synthetic organic resins comprising 1 part of a low-molecular-weight vinyl chloride polymer having an average molecular weight between about 5000 and 16000 and a combined vinyl chloride content in excess of about 60% by weight of the polymer, having dispersed therein as a distinct undissolved solid phase 1 to 6 parts of a relatively high-molecular-weight emulsion-polymerized vinyl chloride polymer having an average molecular weight above about 20,000 and a combined vinyl chloride content in excess of 90% by weight of the polymer and between about 37% and 58% of the weight of said polymers of plasticizer of which less than 70% is a plasticizer leachable in an aqueous soap solution, and the balance is a plasticizer non-leachable in an aqueous soap solution.

3. In the process of manufacturing a multiple ply article of apparel such as collars, cuffs and shirt bosoms wherein an interliner fabric is coated with an adhesive and subsequently composed to a face fabric by heat and pressure, the improvement which comprises coating said interliner fabric with a mixture of separately-polymerized resins constituting a liquid coating composition comprising a distinct undissolved solid disperse phase of 1 to 6 parts by weight of a finely-divided emulsion-polymerized vinyl chloride polymer having an average molecular weight above 20,000, and a combined vinyl chloride content in excess of 90% by weight of the polymer, in a continuous phase of a solution of 1 part of a vinyl chloride polymer having an average molecular weight between 5,000 and 16,000 and a combined vinyl chloride content in excess of about 60% by weight of the polymer, said continuous phase containing a plasticizer in an amount between about 37% and 58% by weight of the total polymer content of which less than

about 70% is a plasticizer leachable in an aqueous soap solution, and the balance is a plasticizer non-leachable in an aqueous soap solution, and removing the solvent from said coating by evaporation.

4. In the process of manufacturing a multiple ply article of apparel such as collars, cuffs and shirt bosoms wherein an interliner fabric is coated with an adhesive and subsequently composed to a face fabric by heat and pressure, the improvement which comprises coating said interliner fabric with a mixture of separately-polymerized resins constituting a liquid coating composition comprising a distinct undissolved solid disperse phase of 1 to 6 parts by weight of a finely-divided emulsion-polymerized vinyl chloride polymer having an average molecular weight above 20,000 and a combined vinyl chloride content in excess of 90% by weight of the polymer, in a continuous phase of a solution of 1 part of a vinyl chloride polymer having an average molecular weight between 5,000 and 16,000 and a combined vinyl chloride content in excess of about 60% by weight of the polymer, in a solvent composed of at least one alkyl ketone having the formula



30 wherein  $R_1$  and  $R_2$  are alkyl groups selected from the class consisting of methyl, ethyl, n-propyl, isopropyl and isobutyl, said continuous phase containing a plasticizer in an amount between about 37% and 58% by weight of the total polymer content of which less than about 70% is a plasticizer leachable in an aqueous soap solution, and the balance is a plasticizer non-leachable in an aqueous soap solution, and removing the solvent from said coating by evaporation.

5. The process according to claim 4 in which the solvent is acetone.

6. An interliner fabric according to claim 1 in which the high molecular-weight emulsion-polymerized vinyl chloride polymer consists of polyvinyl chloride.

7. An interliner fabric according to claim 1 in which the high molecular-weight emulsion-polymerized vinyl chloride polymer is a copolymer of vinyl chloride and vinyl acetate in the ratio of about 95:5, and the low molecular-weight vinyl chloride polymer is a copolymer of vinyl chloride and vinyl acetate in the ratio of about 87:13.

ROBERT H. GILLESPIE.

References Cited in the file of this patent

UNITED STATES PATENTS

| Number    | Name          | Date           |
|-----------|---------------|----------------|
| 2,057,671 | Dreyfus       | Oct. 20, 1936  |
| 2,100,712 | Emmey         | Nov. 30, 1937  |
| 2,245,708 | Patton        | June 17, 1941  |
| 2,325,963 | Lott et al.   | Aug. 3, 1943   |
| 2,329,456 | Campbell      | Sept. 14, 1943 |
| 2,385,879 | Patton        | Oct. 14, 1945  |
| 2,396,125 | Price         | Mar. 5, 1946   |
| 2,431,078 | Powell et al. | Nov. 18, 1947  |
| 2,544,873 | Adams         | Mar. 13, 1951  |